

# UNITED STATES PATENT OFFICE.

FRIEDRICH BÖLLING, OF OBERURSEL, GERMANY, ASSIGNOR OF ONE-HALF TO THE FIRM OF "PROMETHEUS" FABRIK ELEKTRISCHER KOCH- UND HEIZAPPARATE, GESELLSCHAFT MIT BESCHRÄNKTER HAFTUNG, OF FRANKFORT-ON-THE-MAIN, GERMANY.

## INSULATING MATERIAL.

1,123,985.

Specification of Letters Patent.

Patented Jan. 5, 1915.

No Drawing.

Application filed May 31, 1913. Serial No. 770,945.

To all whom it may concern:

Be it known that I, FRIEDRICH BÖLLING, engineer, citizen of Germany, and resident of Oberursel, near Frankfort-on-the-Main, 5 Germany, have invented certain new and useful Improvements in Insulating Materials, of which the following is a specification.

My invention relates to a process for 10 manufacturing heat proof, electric insulating blades, plates, etc., from mica waste and the like.

It is known to produce electric insulating 15 blades, plates, etc., from mica waste, flake mica, split mica, mica powder and the like, these materials being far cheaper than the natural mica, the price of which is constantly increasing, so that it becomes almost prohibitive for certain articles.

20 The mica waste or the like is united to bodies of the form required by using a binding agent and subjecting the mixture to high pressure and high temperature at the same time. The binding agents which have been 25 used or suggested consist of shellac and other carbonaceous materials or of water-glass. All these binding agents can however only be employed, if the insulating bodies so made are not to withstand temperatures higher than say about 150° C. At higher temperatures the carbonaceous 30 materials become soft and charred, develop malodorous vapors and lose their binding and insulating capacities. Waterglass on the other hand gives up its water at said 35 temperature and disintegrates into the form of a powder which no longer possesses any binding qualities and absorbs moisture from the atmosphere, thus unfavorably affecting 40 the insulating properties of the mica bodies to be produced.

Now, on the contrary to the methods referred to before, my process has for its object the manufacture of electric insulating 45 blades, plates, etc., from mica waste and the like, which are capable of withstanding temperatures up to 900° C. without any deleterious effect and without being inferior to the natural mica as regards insulating 50 power, hardness and cleavage. Such insulating bodies are especially qualified for use with electric cooking vessels, flat irons and similar apparatus, where they have to with-

stand, as is well known, temperatures up to 400° C. and more, for some considerable 55 time and not only temporarily.

In addition to the well known steps to combine the initially loose mica particles by means of a binding agent under an elevated temperature and high pressure, my new 60 process offers the distinctive feature, that the mixture of mica waste or the like and binding agent is heated from 500° to 950° C. and that a binding agent is used consisting of an inorganic compound and having 65 a melting point from 500° to 950° C. Such compounds are for instance employed as fluxes in the manufacture of ceramic wares. As an example, of these may be mentioned a flux containing boron, silicon and lead. 70 Higher temperatures are not advisable, as they destroy valuable qualities of the mica, and also because they are fully sufficient for all practical purposes of the insulating bodies to be produced.

75 The mica waste and the like may be made up to form plates and so forth according to the present invention, by causing separate thin mica layers to be covered with the flux material and to be laid one on another, as 80 customary in the manufacture of micanite, after which they are submitted simultaneously to great pressure and to a high temperature. Any suitable pressure may be employed, and the temperature will be just sufficiently high to melt completely the binding or fluxing material without deleteriously affecting its qualities or those of the mica. In another method of working, a layer of 85 thin mica is covered with the binding or fluxing material and then mica dust, which is a very cheap substance, is strewed over the surface. When the desired thickness 90 has been built up a covering sheet of split mica is laid over the top and the whole is 95 pressed and heated as above mentioned. A number of successive layers made in this way may be used to form a plate or block of any desired thickness.

I claim:

100 1. An insulating material of the character described, consisting of mica flakes pasted together under high pressure by and while heating to a high temperature an inorganic fluxing material having a melting point between 500 and 950° C. and not being de-

stroyed when heated to this temperature substantially as and for the purpose set forth.

2. An insulating material of the character described consisting of mica flakes pasted together under high pressure by a fluxing material containing boron, silicon, and lead and having a melting point between 500 and 950° C. substantially as and for the purpose set forth.

3. The process of making an insulating material of the character described, which consists in mixing mica flakes with an inorganic fluxing material having a melting point between 500 and 950° C. and not being destroyed when heated to this temperature heating the mass to said temperatures and subjecting it at the same time to high

pressure, substantially as and for the purpose set forth.

20

4. The process of making an insulating material of the character described, which consists in mixing mica flakes with a fluxing material containing boron, silicon and lead and having a melting point between 500 and 950° C. heating the mass to said temperatures, and subjecting it at the same time to high pressure, substantially as and for the purpose set forth.

25

In testimony whereof I affix my signature in presence of two witnesses.

FRIEDRICH BÖLLING.

Witnesses:

JEAN GRUND,  
CARL GRUND.